

Nov. 4, 1952

R. LEVI

2,616,840

RHENIUM PLATING

Filed Nov. 12, 1948

2 SHEETS—SHEET 1



FIG. 1



FIG. 2

INVENTOR

ROBERTO LEVI  
BY *Frederick M. Magel*  
AGENT

Nov. 4, 1952

R. LEVI

2,616,840

RHENIUM PLATING

Filed Nov. 12, 1948

2 SHEETS--SHEET 2



FIG-3a

FIG-3b

FIG-3c

FIG-3d

INVENTOR

ROBERTO LEVI

BY *Robert M. Levy*

AGENT

## UNITED STATES PATENT OFFICE

2,616,840

## RHENIUM PLATING

Roberto Levi, New York, N. Y., assignor to Philips Laboratories, Inc., Irvington-on-Hudson, N. Y.

Application November 12, 1948, Serial No. 59,674

5 Claims. (Cl. 204—37)

## 1

My invention relates to a method for plating rhenium upon a base metal giving a durable, impervious rhenium layer.

Rhenium is an element occurring in minutely small amounts throughout the surface of the earth. It is a hard bright metal when in a massive state, resembling tungsten or rhodium. Further characteristics of rhenium are its extremely high melting point, a high resistance to attack by hydrochloric acid, a volatilization less than tungsten in vacuo, and an electron emissivity approximately equivalent to tungsten; it is a desirable plating material.

My invention is particularly advantageous to connection with plating rhenium upon other less expensive metals, giving such other metals a hard, massive coating of rhenium. As I have obtained especially advantageous results using refractory metals, for example tungsten and molydenum, as base metals, I shall describe the invention in this connection. However, the invention is not limited to the use of tungsten and molydenum or refractory base metals, but extends to other metals such as platinum, rhodium, nickel, chromium and the like.

The electrodeposition of rhenium, *per se*, is known. With the proper control of such factors as current density, hydrogen ion concentration, temperature, etc., it has been possible to obtain a massive electrodeposition of rhenium from various aqueous plating solutions containing compounds of rhenium. Such known processes have in common at least two serious objections. The first is the rapid oxidation of the deposited rhenium after a few days of exposure to moist air at room temperature. Such oxidation converts the entire deposited layer to perrhenic acid. The second objection is to be found in the fact that even if a stable plating could be made by known processes, an ordinarily thick electrodeposition of rhenium will introduce internal stresses in the deposited layer rendering the deposit extremely brittle and weak at temperatures above room temperature.

It is an object of my invention to provide an improved method for the plating of rhenium which is free from the objections found in the known methods. Another important object of my invention is to provide rhenium plated articles of practical use, such as a cathode emitter for electron discharge tubes comprising a layer of plated rhenium upon a refractory base metal such as tungsten. A further object of my invention is to provide articles of pure rhenium such as seamless hollow cylinders, foil and ribbon.

## 2

Other objects and advantages of the invention will be apparent from the following description and from the accompanying drawings.

Fig. 1 illustrates schematically one form of apparatus for electrodepositing of rhenium.

Fig. 2 shows one form of apparatus for preparing rhenium plating in accordance with the invention.

Fig. 3a shows an X-ray diffraction photograph indicating the crystallographic structure of rhenium and the characteristic lines thereof.

Fig. 3b shows an X-ray diffraction photograph of the crystallographic structure of the element tungsten.

Fig. 3c shows an X-ray diffraction photograph immediately after plating of rhenium upon a base of tungsten.

Fig. 3d shows an X-ray diffraction photograph of plated rhenium on the base of a tungsten metal after treatment in accordance with the method of the invention.

Referring to Fig. 1, a base metal cathode, for example of tungsten to be plated, is cleaned and immersed in an electroplating solution 5. This electroplating solution 5 may contain for example: potassium perrhenate,  $KReO_4$ , 11 grams per liter; concentrated sulphuric acid,  $H_2SO_4$ , the solution having a  $pH=0.9$ . The temperature of the solution maybe about  $25^\circ$  to  $45^\circ$  C. Other sulphate baths are known utilizing various aqueous solutions of rhenium compounds and indeed other baths such as phosphate and alkaline baths maybe employed in accordance with known procedures, with the proper adjustment of hydrogen ion concentration, temperature, etc. Element 1 shows an anode which maybe made of platinum. The cathode and anode, 2 and 1 respectively, are connected as electrodes in an electric circuit, in accordance with the ordinary techniques of plating, including a source of direct current potential 4, and a current indicating device 3.

The plating operation is continued at a given current density depending upon the solution or bath used until plated layer is deposited preferably having a thickness about  $.0001''$  to  $.0003''$ . In the electroplating solution heretofore stated, a current density of 10 to 14 amp./dm<sup>2</sup> is satisfactory. The plated cathode is then removed from the electroplating solution.

Other sulphate plating baths which maybe employed successfully include: perrhenic acid,  $HReO_4$ , 20 grams per liter; concentrated sulphuric acid to bring the solution to  $pH=0.7$  to 1.2; the temperature between  $25^\circ$  to  $30^\circ$  C.; cur-

rent density, 10 to 15 amp./dm<sup>2</sup>. Another sulphate bath may consist of potassium perrhenate, KReO<sub>4</sub>, 10 to 25 grams per liter; concentrated sulphuric acid to bring the solution to pH=0.80 to 1.00; the temperature between 25° to 45° C.; current density 10 to 16 amp./dm<sup>2</sup>.

A phosphate bath maybe used, for example, potassium perrhenate, KReO<sub>4</sub>, 3 grams; phosphoric acid, sp. gr. 1.7, 7.0 cc.; sodium phosphate, Na<sub>2</sub>HPO<sub>4</sub>, 16.5 grams; water, 250 cc.; temperature between 80°-90° C.; pH at 90° C., 2.282; pH at 80° C., 1.743; and current density from 13 to 17 amp./dm<sup>2</sup>.

Fig. 2 shows a further step in the process according to the invention. The cathode 2, now plated, is introduced into a reducing atmosphere 6, within a suitable enclosure 7. Such a reducing atmosphere may be composed by way of example, of hydrogen. While the cathode 2 is within the reducing atmosphere the temperature of the cathode is raised to a high temperature for a short period of time. I have found a temperature of 1000° C. to be satisfactory for the plating of refractory metals; but the melting point of the metal to be plated must be considered. The foregoing may be easily accomplished when cathodes having a uniform cross section, by introducing a source of electric energy 8, at each end of the plated cathode introducing a sufficient current flow in the cathode to cause it to reach the desired temperature. In the case of cathodes of other shapes, induction or furnace heating has been found desirable.

After the cathode has been fired in accordance with the foregoing, it is returned to the electroplating process for further electrodeposition as shown in Fig. 1. The entire process of electrodeposition and heat treatment, as outlined, is repeated until a layer of rhenium having the desired thickness has been obtained. The plating of rhenium in relatively thin layers as described and the subsequent firing apparently serves to alter the crystallographic structure of the plated rhenium upon the base metal. Simultaneously the objectionable internal stresses that I found when a large deposit of rhenium is plated and fired are eliminated. These stresses will cause a failure of the plated material.

The effect of the plating process may be studied by X-ray diffraction analysis. Massive rhenium, when subject to X-ray diffraction analysis, displays a spectra of lines as illustrated in Fig. 3a. With the plating of rhenium upon a given base metal, the plating displays a structure which is apparently non crystalline as indicated by the lack of lines, Fig. 3c. It is this structure that is obtained when rhenium is plated without the process as described in my invention. This plating is subject to the attack of moist air and the subsequent oxidation of the plated rhenium to perrhenic acid. However, in comparison with an X-ray diffraction photograph of tungsten, as shown in Fig. 3b, it may be seen that even the non crystalline electrodeposition of Fig. 3c upon the base metal tungsten shows none of the characteristic lines of tungsten perceptible through the plated layer.

Upon the heat treatment of the plated cathode in accordance with the procedure heretofore described, the plated rhenium layer appears by X-ray diffraction as shown in Fig. 3d. The non crystalline structure of the electrodeposition has disappeared and is replaced by the charac-

teristic crystalline structure first seen in the X-ray diffraction photograph of massive rhenium, per se, Fig. 3a. It is to be noted that still no characteristic lines of tungsten may be found visible through the plated layer of rhenium after treatment; indicative of the fact that a massive coating of rhenium has been deposited on the base metal, and that the coating has not split to reveal the underlying tungsten base.

Such articles as seamless hollow cylinders, foil and ribbon may be made by plating a suitably shaped base metal according to the invention. A base metal for this purpose should have a melting point above 1000° C. and should be soluble in reagents that do not affect rhenium. For example such a reagent may be hydrochloric acid, HCl. Subsequent immersion of the plated article in hydrochloric acid will erode the base metal, leaving the desired article of pure rhenium.

Having thus described my invention, what I claim as new and desire to secure by Letters Patent of the United States is:

1. The process of plating a predetermined thickness of rhenium upon a tungsten base, comprising the steps of electrodepositing on said tungsten base a first deposited layer of rhenium having a non crystalline structure and a thickness substantially between 0.0001" to 0.0003", 25 heating the said electrodeposited rhenium in a reducing atmosphere to a temperature of approximately 1000° C. and converting the said first deposited layer to rhenium having a crystalline structure, electrodepositing on the first crystalline rhenium layer a second deposit of rhenium, heating said second deposit of rhenium and converting the said second deposit to rhenium having a crystalline structure, and repeating the said electrodeposition and heating 30 steps until the predetermined thickness of electrodeposited crystalline rhenium is produced.

2. A method of forming on a base of refractory metal a covering of substantial thickness of pure stable rhenium in crystalline form having an X-ray diffraction pattern containing all of the characteristic lines of crystalline rhenium which comprises the steps of electro-depositing on the base a thin layer of amorphous rhenium, transforming the amorphous rhenium layer into a layer of crystalline rhenium by heating the same in a reducing atmosphere at a temperature at which the rhenium crystallizes without melting, and successively repeating the steps until a coating of crystalline rhenium of substantial thickness is obtained.

3. A method of forming on a base of tungsten a stable covering of substantial thickness of pure stable rhenium in crystalline form having an X-ray diffraction pattern containing all of the characteristic lines of crystalline rhenium which comprises the steps of electro-depositing on the tungsten base a thin layer of amorphous rhenium, transforming the amorphous rhenium layer into a layer of crystalline rhenium by heating the same in a reducing atmosphere at a temperature at which the rhenium crystallizes without melting, and successively repeating the steps until a coating of crystalline rhenium of substantial thickness is obtained.

4. A method of forming on a base of tungsten a stable covering of substantial thickness of pure stable rhenium in crystalline form having an X-ray diffraction pattern containing all of the characteristic lines of crystalline rhenium which

comprises the steps of electro-depositing on the tungsten base a thin layer of amorphous rhenium, transforming the amorphous rhenium into a layer of crystalline rhenium layer by heating the same in a reducing atmosphere at a temperature of about 1000° C. and successively repeating the steps until a coating of crystalline rhenium of substantial thickness is obtained.

5. A method of forming on a base of refractory metal a covering of substantial thickness of pure stable rhenium in crystalline form having an X-ray diffraction pattern containing all of the characteristic lines of rhenium which comprises the steps of electrodepositing on the base a thin layer of amorphous rhenium, transforming the amorphous rhenium into a layer of crystalline rhenium by heating the same in a reducing atmosphere at a temperature of about 1000° C and successively repeating the steps until a coating of crystalline rhenium of substantial thickness is obtained.

ROBERTO LEVI.

#### REFERENCES CITED

The following references are of record in the file of this patent:

#### UNITED STATES PATENTS

| Number       | Name             | Date          |
|--------------|------------------|---------------|
| 1,565,724    | Fonda            | Dec. 15, 1925 |
| 1,838,273    | McBride          | Dec. 29, 1931 |
| 2,138,573    | Fink et al.      | Nov. 29, 1938 |
| 10 2,149,656 | Armstrong et al. | Mar. 7, 1939  |
| 2,195,499    | Schofield        | Apr. 2, 1940  |
| 2,512,141    | Ma et al.        | June 20, 1950 |

#### OTHER REFERENCES

- 15 Mellor, Comprehensive Treatise on Inorganic and Theoretical Chemistry, vol. 12, (1932), p. 468.  
 Fink et al, Transactions Electrochemical Society, vol. 66, (1934), pp. 471-474.
- 20 Holeman, Zeitschrift fur anorganische und Allgemeine Chemie, vol. 202, (1931), pp. 277-291.  
 Young, Metal Industry, vol. 34, (1936), pp. 176-177.